

## UNITED STATES PATENT OFFICE

2,551,124

LUBRICATING COMPOSITIONS AND  
ADDITIVES THEREFOR

William Helmore, Kingston Hill, England, assignor to C. C. Wakefield & Company Limited, London, England, a British company

No Drawing. Application February 25, 1948, Serial No. 10,927. In Great Britain February 27, 1947

4 Claims. (Cl. 252—33)

1

The present invention comprises improvements in or relating to lubricating compositions and additives therefor, and relates more especially though not exclusively to lubricating compositions for use in internal combustion engines under conditions of high temperature to lubricate parts subject to large mechanical stresses.

In his previous British Patent Specifications Nos. 398,222 and 423,441 the inventor has shown that lubricating compositions formed by the addition to a lubricating oil of small amounts of organic compounds of tin and of organic compounds of chromium respectively, results in a marked increase in resistance to oxidation of the lubricant and reduces the formation of gum and other deposits during use. The use of chromium or an organic compound thereof in a lubricating oil together with one or more other substances such as an organic compound of tin and/or lead has also been proposed in British Patent Specification No. 431,066.

According to the present invention a lubricating composition comprises a small proportion of the organo-metallic petroleum sulphonate of tin or chromium.

The inventor has found that such lubricating compositions have particularly good resistance to oxidation under conditions of use in an internal combustion engine and have also good anti-corrosive properties, and do not form excessive deposits in the piston ring grooves or promote lacquering of the pistons.

The resistance to physical wear, oxidation or other corrosion of metallic tin and chromium when applied as a coating to pistons and cylinders respectively of internal combustion engines has, subsequently to the proposals of the said prior specifications, become well known and established and the subject of accepted use in engines of high quality. The inventor has also found that some analogous resistance to corrosive or abrasive wear of piston and cylinder surfaces may be obtained in an internal combustion engine by the use of tin and/or chromium petroleum sulphonates in the lubricant for the engine.

Accordingly, the present invention provides also a lubricating composition comprising a lubricating oil base in which is incorporated a minor proportion of organic compounds of both chromium and tin whereof at least one of such organic compounds is a petroleum sulphonate. Conveniently such a lubricating composition comprises a minor proportion of chromium or tin petroleum sulphonate and a further organic com-

2

ound other than a petroleum sulphonate of tin or chromium respectively.

It is to be understood also as within the present invention to employ in a lubricating oil base 5 chromium and tin petroleum sulphonates in admixture and/or other organic compounds of chromium and tin in admixture. It is to be understood further that all compounds of chromium and tin the use of which is contemplated 10 by the present invention are those which are soluble in the lubricating oil base.

Examples of the organic compounds of chromium and tin (other than the petroleum sulphonates) referred to above are conveniently afforded by the oleates, naphthenates or substituted phenolates, and such compounds and the sulphonates referred to above may each be employed in any desirable proportion for example, to an extent of from 0.05% to 2.0% by weight in 20 the composition.

According to one example of the invention a lubricating composition suitable for use in a conventional petrol engine is afforded by a lubricating oil base in which there is incorporated 0.1% 25 by weight of chromium and/or tin petroleum sulphonate together with 0.4% by weight of other organic tin and/or chromium compound respectively. In other examples a similar relative proportion by weight of such compounds may 30 be employed.

Conveniently a lubricating composition provided in accordance with the invention comprises also a small proportion of alkali (e. g. sodium) petroleum sulphonate and/or alkaline earth (e. g. 35 calcium) petroleum sulphonate. Conveniently also the alkali and/or alkaline earth petroleum sulphonates are selectively included in the composition to exclude such compounds of a pronounced corrosive nature. Apart from benefits 40 found in normal running of an engine with use of the lubricating compositions now proposed, the inclusion in the latter of the said sodium and calcium petroleum sulphonates, particularly in their selectively refined form, have been found to 45 afford protection to the cylinders and other parts of the engine subject to corrosion during periods of storage of the engine or when the latter is otherwise stationary.

The lubricating composition may comprise a 50 proportion of from 0.01% to 2.0% by weight of added petroleum sulphonate and preferably contains about 1.0% by weight of the organo-metallic petroleum sulphonate of chromium and/or tin with a proportion of selectively included alkali or alkaline earth petroleum sul-

phonate. The chromium and tin petroleum sulphonates when employed in admixture however may be present in relative proportions by weight of approximately 1 to 4. For example, the amount of chromium petroleum sulphonate may range from 0.1% to 0.3% and the amount of tin petroleum sulphonate may range from 0.4% to 1.2%.

Other known lubricant additives such as V. I. improvers, pour-point depressants, or materials for increasing the film rupture strength of the composition and/or other anti-oxidant and/or detergent additives may also be added to the lubricating composition provided by the invention. Thus a small proportion of tri-ortho-cresyl phosphate or of tributyl phosphite may be employed in a lubricating oil in conjunction with the tin and/or chromium petroleum sulphonate in order also to enhance the film rupture strength and other properties of the composition.

The present invention also includes a process of producing an additive material for incorporation in a lubricating composition as referred to above from petroleum sulphonic acids, for example, by reacting the alkali or alkaline earth petroleum sulphonates with appropriate salts of chromium and/or tin. The latter's salts may be chrome alum or chromium sulphate or chromium chloride, or other suitable inorganic salts of chromium, or a mixture of suitable chromium salts, and/or stannous chloride or other suitable inorganic salt or salts of tin, and the chromium and tin salts may also be employed in admixture in proportions to yield under the reaction conditions chromium and tin petroleum sulphonates in a desired relative proportion by weight. Conveniently, the reaction components and/or conditions are adjusted to produce a desired proportion of unreacted alkali (e. g. sodium) or alkaline earth (e. g. calcium) petroleum sulphonate in the reaction product. The amount of the sodium or calcium petroleum sulphonate in the final lubricating oil composition may range from 0.1% to 1.0% by weight. The reaction may be carried out in aqueous and/or alcoholic solution, and in the latter case according to one specific method stannous chloride and/or chrome alum are added to an alcoholic solution of calcium petroleum sulphonate in equivalent molecular proportions. The mixture is vigorously agitated and the resultant precipitated calcium sulphate for example, filtered off and the alcohol evaporated.

The invention includes also a lubricant additive material for use in the production of a lubricating composition as referred to above comprising the product of a reaction as described in the immediately preceding paragraph. The tin or chromium petroleum sulphonates or mixtures thereof so obtained may be viscous liquids or solids according to the nature of the petroleum sulphonates or sulphonic acids originally employed. The compounds produced in this way are also oil soluble and filter passing when in oil solution, the liquid compounds, however, being more readily soluble.

It will be appreciated that the original sulphonic acids, from which the chromium or tin compounds are now to be derived, are the oil soluble, so-called "mahogany acids." Separated oil soluble sulphonic acids are commercially available in products of the sulphonation of mineral oil of a paraffinic or naphthenic nature and more usually after neutralisation of the free acids by caustic soda or lime to produce either sodium or calcium petroleum sulphonates in admixture with mineral oil. Such a commercially

available material, for example, has been found to contain some 50 to 55% of sodium petroleum sulphonate.

#### Example 1

In one example of the invention 500 grams of the latter commercially available material was mixed with 150 grams of chrome alum and the mixture heated with 2.5 litres of water at a temperature of 100° C. for 18 hours. After subsequent evaporation of the water the residue was then twice extracted with 2.5 litres of benzene maintained at its boiling point for 1 hour. After filtration through a streamline filter the benzene solution gave the following analysis:

|                           | Per cent by weight |
|---------------------------|--------------------|
| Total sulphonates and oil | 6.0                |
| Chromium                  | 0.07               |

These figures correspond to a conversion of approximately 25% of the sodium petroleum sulphonate to the corresponding chromium compound. The probable composition of the material after evaporation of the benzene is:

|                               | Per cent by weight |
|-------------------------------|--------------------|
| Chromium petroleum sulphonate | 10 to 15           |
| Sodium petroleum sulphonate   | about 40           |
| Lubricating oil               | 45 to 50           |

#### Example 2

In a further example of the invention giving a higher yield of chromium petroleum sulphonate, 250 grams of sodium petroleum sulphonate was mixed with 40 grams of chromic chloride and 2 litres of industrial alcohol and heated under reflux conditions for 6 hours. The alcohol was then boiled off and 2 litres of benzene added. The mixture was then boiled for 2 hours and after cooling the resulting solution was filtered through a stream line filter. The benzene was then boiled off and the resulting compound has the composition on an oil free basis of:

|                                       | Per cent by weight |
|---------------------------------------|--------------------|
| Chromium petroleum sulphonate         | 71                 |
| Unreacted sodium petroleum sulphonate | 29                 |

#### Example 3

In a further example of the invention 300 grams of calcium petroleum sulphonate and 150 grams of chrome alum were mixed with 3 litres of aqueous alcohol and refluxed for six hours. The alcohol was then boiled off, 500 ccs. of benzene added and brought almost up to the boiling point. The benzene solution so obtained was then passed through a streamline filter and the benzene evaporated off. The resulting product was found to consist of 70% chromium petroleum sulphonate and 30% unreacted calcium petroleum sulphonate.

#### Example 4

In another example of the invention 600 grams of the commercial sodium petroleum sulphonate referred to above was mixed with 85 grams of stannous chloride and heated in the presence of 1800 cc. of industrial alcohol for a period of nine hours in a water bath with the use of a reflux condenser. After subsequent removal of the alcohol by distillation the residue was then twice heated in succession with 300 ccs. of benzene for 1 hour. After passage through a streamline filter the benzene solution was found to include:

|                           | Per cent by weight |
|---------------------------|--------------------|
| Total sulphonates and oil | 70                 |
| Tin                       | 0.5                |

These figures correspond to a conversion of approximately 65% of the sodium petroleum sulphonate to the corresponding tin compound. The probable composition of the material after evaporation of the benzene is:

| Per cent by weight          |       |
|-----------------------------|-------|
| Tin petroleum sulphonate    | 45    |
| Sodium petroleum sulphonate | 10-15 |
| Lubricating oil             | 40-45 |

It will be noted that in the four examples given above the desired material may be obtained as a clear solution in benzene and may be used as such.

By way of examples of processes for the production of tin and chromium petroleum sulphonates giving high yields of the latter materials with very little or no unreacted alkali petroleum sulphonate in the final product, the following two further examples are given. In both these examples a commercially available sodium petroleum sulphonate material was employed having an approximate content by weight of—

38% sodium petroleum sulphonate  
52% oil  
10% water, alcohol and sodium sulphate

*Example 5*

4 lbs. of the sodium petroleum sulphonate material were added to about 3½ gallons of water and stirred well while heating to 90° C. to produce a fluid milky solution. ½ lb. of tin chloride ( $\text{SnCl}_2 \cdot 2\text{H}_2\text{O}$ ) was dissolved in 500 ccs. of cold water and added to the heated milky sodium petroleum sulphonate solution, stirring being continued. An oil concentrate of tin petroleum sulphonate was precipitated and settled at the bottom of the reaction vessel.

After cooling the water layer was easily decanted or siphoned off from the very viscous precipitate which was washed by adding 1 gallon of water and heating to the boiling point while again stirring well. 4 lbs. of mineral oil were now stirred in to produce a concentrate which was lighter than water, separation being effected by passing the whole mixture through a De Laval centrifuge.

The product, free from insoluble matter, was then freed from a residual 4% of water by heating to 250° F. in a current of air. A 96% yield of 7 lbs. 6½ ozs. was obtained having an approximate composition of—

| Per cent                 |    |
|--------------------------|----|
| Tin petroleum sulphonate | 21 |
| Mineral oil              | 79 |

Analysis of this product gave the results:

| Per cent              |      |
|-----------------------|------|
| Tin (Kjeldahl method) | 2.74 |
| Sodium                | Nil  |
| Ash                   | 3.56 |

*Example 6*

4 lbs. of the sodium petroleum sulphonate material were added to about 4 gallons of water and mixed while heating to 90° C. A hot solution at 90° C. of 13 oz. of chrome alum in ½ gallon of water was then added while stirring and the mixture allowed to stand overnight. Water was then decanted from the viscous oil solution which had settled in the reaction vessel and which was washed with a further 2 gallons of water by heating to boiling point and stirring well. After cooling the water was again decanted and the remain-

ing product finally dried by heating to 250° F. in a current of air. Centrifuging was considered unnecessary in view of the appearance of the product but may be desirable under certain circumstances.

The product represented an 87% yield of 3 lbs. 2 ozs. having an approximate composition of—

|                               | Per Cent     |
|-------------------------------|--------------|
| Chromium petroleum sulphonate | 31.5         |
| Sodium petroleum sulphonate   | 6 to 8       |
| Mineral oil                   | 60.5 to 62.5 |

Analysis of the product gave the results:

|          | Per Cent |
|----------|----------|
| Chromium | 1.81     |
| Sodium   | 0.47     |
| Ash      | 3.79     |

If desired, chromium and tin petroleum sulphonates may be prepared in admixture by the simultaneous reaction of chrome alum, chromium sulphate, or chromium chloride, or any other suitable inorganic salt of chromium, or any preferred mixture of such salts, and stannous chloride, or other suitable inorganic salt or salts of tin with the first mentioned commercial sodium petroleum sulphonate or an equivalent material, the proportions of chrome alum and/or said other chromium salt or salts and stannous chloride or other preferred salt or salts employed together for this reaction preferably being such as to secure a desired content of chromium and tin petroleum sulphonates in relation to one another in the reaction product. A similar procedure may also be adopted, if desired, in the preparation of mixed chromium and tin petroleum sulphonates free from alkali or alkaline earth sulphonates by production from the free petroleum sulphonic acids. The latter may be obtained, for example, by the action of hydrochloric acid on the sodium or calcium sulphonates. The chromium and tin compounds may also be separately produced in this way free from sodium or calcium sulphonates. Such processes with the use of free sulphonic acids however, are more costly and troublesome than those described above in which the stable unreacted sodium and/or calcium sulphonate are also present in the reaction product. By variation of the latter process, for example as regards the temperature or duration, at or for which the reaction is effected or by the choice of starting materials, a desired content of such sodium and/or calcium sulphonate in the reaction product may also be secured, and it may sometimes be advantageous to effect a reduction in the quantity of the sodium sulphonate produced with the corresponding chromium compound as in the second specific example referred to above, without proceeding to a substantially complete conversion of the sodium petroleum sulphonate as described in Examples 5 and 6.

Proportions of from 0.05% up to 2.0% by weight of the chromium and/or tin compounds are found to be advantageously employed in a lubricating composition, and in a particular mixture 0.1% of the chromium compound and 0.4% of the tin compound is found to be especially desirable either when used alone or with less than an equal quantity of the unreacted sodium and/or calcium petroleum sulphonate.

Of the known agents which may also be added to lubricating compositions (e. g. for imparting anti-oxidant or detergent properties and/or for increasing the film rupture strength) it has been

found particularly satisfactory to include also an aromatic hydroxy-substituted thioether and/or di- or poly-sulphide compound as described in British Specifications Nos. 455,235 and 561,898 and/or a phosphite or thiophosphite ester thereof as described in British Specification No. 574,445. Alternatively or in addition tri-cresyl phosphate may also be included in the composition. Such compounds may be employed in the composition to an extent of about 0.1% to 1.0% by weight.

Again the additives proposed by the present invention may also be employed, for example, and with advantage to replace a metal soap where the latter has been included in a lubricating composition. The organic compound of tin employed in the compositions proposed in the inventor's prior British Patent Specification No. 548,390 may thus be replaced by the tin and/or chromium petroleum sulphonates now proposed, while the latter may also be employed in place of the metal soap in the compositions described in the inventor's prior British Patent Specification No. 510,244.

Lubricating compositions provided by the invention have increased resistance to oxidation and sludge formation at all temperatures and also show a reduced tendency for the production in use of gummy deposits by thermal decomposition. The compositions also have improved detergent properties.

The resistance to corrosive or abrasive wear of cylinder and piston surfaces, as well as bearing surfaces referred to as analogous to that secured by the application of a metallic coating of chromium and tin respectively, is also secured to a remarkable extent. It is also found that although commercial calcium and sodium petroleum sulphonates separately used in a lubricating oil produce markedly increased corrosion, sodium and calcium petroleum sulphonates are capable of use with chromium and/or tin petroleum sulphonates without a marked increased of corrosion and with improved properties of oxidation resistance and detergency imparted to the lubricant.

The surprising absence of increased corrosion under the latter conditions is particularly true in the case of the presence of sodium or calcium petroleum sulphonate as an unreacted residue in the preparation of the chromium and/or tin compounds. This result is apparently due to a selective reaction of the chromium and/or tin salts with the less stable and more corrosive sodium or calcium sulphonate molecules so that the residual alkali or alkaline earth sulphonate molecules in the reaction product are of a more desirable, more stable and less corrosive nature. It is accordingly preferred to include in the lubricating compositions an alkali and/or alkaline earth petroleum sulphonate of this nature which may be derived in the manner indicated.

Comparative laboratory test results were secured in:

(A) The standard Air Ministry oxidation test.  
(B) A corrosion test in which lead or mild steel test pieces were rotated at 700 R. P. M. in contact with the oil and only partly immersed during heating of the oil to 180° C. for 12 hours, loss in weight of the test pieces being recorded and polished copper being present in the oil to act as catalyst.

(C) A filtration test in which an oil sample was passed through a closely packed and highly efficient filter of the streamline type, the tin

and/or chromium content of the oil sample being determined before and after filtration.

The tests were conducted on three oil samples as follows:

- 5 (1) A solvent refined lubricating oil without additives viscosity 489 Redwood No. 1 at 100° F. (120 centistokes) and viscosity index of 93.
- (2) The lubricating oil of sample 1 to which 0.4% by weight of the commercial sodium petroleum sulphonate first referred to above had been added.
- (3) The lubricating oil of sample 1 containing 0.1% by weight of chromium petroleum sulphonate, 0.4% by weight of tin petroleum sulphonate and 0.35 to 0.4% by weight of sodium petroleum sulphonate left as unreacted residue in the production of the chromium and tin compounds.

Test results secured were as follows:

| Oil Sample                      | 1        | 2          | 3     |
|---------------------------------|----------|------------|-------|
| 25 Viscosity at 100° F.:        |          |            |       |
| Redwood No. 1 (Secs.)           | 487      | 491        | 492   |
| Centistokes                     | 120      | 121        | 121   |
| Carbon Residue, per cent wt.    | 0.2      | 0.38       | 0.3   |
| 30 (A) Oxidation Test:          |          |            |       |
| Viscosity after Oxidation (Cs.) | 216      | 175        | 206   |
| Viscosity Ratio                 | 1.8      | 1.45       | 1.7   |
| Carbon Residue after Oxidation  | 1.7      | 1.28       | 1.9   |
| Carbon Residue increase         | 1.5      | 0.9        | 1.6   |
| 35 (B) Corrosion Test:          |          |            |       |
| Weight loss (mg.):              |          |            |       |
| Lead                            | 150      | about 500  | 5.0   |
| Steel                           | 11.0     | above 30.0 | 0.8   |
| (C) Filter Test:                |          |            |       |
| Tin before filtration           | per cent |            | 0.065 |
| Tin after filtration            | do       |            | 0.064 |
| Per cent loss                   |          |            | Nil   |
| Chromium before filtration      | per cent |            | 0.003 |
| Chromium after filtration       | do       |            | 0.003 |
| Per cent loss                   |          |            | Nil   |

40 The lubricating composition provided by the invention includes additives of a highly oil soluble nature capable in solution in oil in the desired proportions of passing a stream line filter without the effective removal of any of the additive material. Since the latter act as wetting agents they also confer benefit particularly in use in internal combustion engines in securing the spread and retention of an oil film on cylinder and other rubbing surfaces especially when such engines are left stationary after running. This is particularly so in the case of lubricating compositions provided by this invention containing sodium petroleum sulphonate and/or calcium petroleum sulphonate in the mixture, in that at ordinary temperatures e. g. during storage of the engine, the last-mentioned sulphonates act as rust preventers and generally as corrosion inhibitors.

45 Lubricating compositions provided in accordance with the present invention had also been subject to practical tests under operating conditions in a conventional type of single cylinder test engine. One such test was conducted with a lubricating composition in which there was incorporated 1.2% by weight of tin petroleum sulphonate as produced in Example 4 (and thus including a proportion of unreacted sodium petroleum sulphonate) and 0.3% of chromium petroleum sulphonate as produced in Example 3 (and thus including a proportion of unreacted calcium petroleum sulphonate). After the test run the engine was found to have a very clean piston and no varnish or lacquer deposit on the bearings. Bearing corrosion showed a loss in weight of bearing parts of 28 milligrams as com-

pared with a loss of 153 milligrams for a similar test run with the unmodified lubricating oil in which the tin and chromium petroleum sulphonates were incorporated.

Other satisfactory engine test results have been obtained with the use in a lubricating oil of tin and/or chromium petroleum sulphonate in conjunction with other organic compounds of chromium and/or tin respectively, confirming the benefits indicated above. Other known organic compounds, such as mercaptobenzothiazole, have also been included with advantage in such compositions. Good results have thus been obtained with the use in a lubricating composition of from 0.1% to 0.2% of tin petroleum sulphonate and 0.4% to 0.8% of chromium oleate and, alternatively, with the use of from 0.1% to 0.2% of chromium petroleum sulphonate with 0.4% to 0.8% of tin oleate. A number of laboratory and engine tests have been made also to confirm the advantages secured in particular with the use of tin petroleum sulphonate in conjunction with a suitable organic chromium compound, for example in proportions corresponding to those suggested for tin petroleum sulphonate and chromium oleate.

I claim:

1. A lubricating composition, which comprises, a mineral lubricating oil base in which is incorporated between 0.05% and 2% by weight of tin petroleum sulphonate and between 0.05% and 2% by weight of chromium petroleum sulphonate.

2. A composition in accordance with claim 1 in which the amount of chromium petroleum sulphonate is between 0.1 and 0.3% and the amount of tin petroleum sulphonate is between 0.4% and 1.2%.

3. A composition in accordance with claim 1 which also contains between 0.1% and 1.0% of a sulphonate selected from the group consisting of sodium petroleum sulphonate and calcium petroleum sulphonate.

4. A composition in accordance with claim 1 which also contains between 0.35% and 0.4% sodium petroleum sulphonate.

WILLIAM HELMORE.

#### REFERENCES CITED

The following references are of record in the file of this patent:

#### UNITED STATES PATENTS

| Number    | Name       | Date          |
|-----------|------------|---------------|
| 2,125,305 | Murphy     | Aug. 2, 1938  |
| 2,125,936 | Liberthson | Aug. 9, 1938  |
| 2,234,005 | Loane      | Mar. 4, 1941  |
| 2,261,047 | Asseff     | Oct. 28, 1941 |
| 2,266,325 | Lazar      | Dec. 16, 1941 |
| 2,367,470 | Neely      | Jan. 16, 1945 |
| 2,410,652 | Griffin    | Nov. 5, 1946  |

#### FOREIGN PATENTS

| Number  | Country       | Date          |
|---------|---------------|---------------|
| 431,066 | Great Britain | July 1, 1935  |
| 510,244 | Great Britain | July 28, 1939 |